

## UNITED STATES PATENT OFFICE.

GEORGE SCHELLHAAS, OF FRANKENTHAL-PFALZ, GERMANY.

## PROCESS FOR MANUFACTURING SOLID CORK BODIES AND THE LIKE.

No Drawing.

Application filed May 11, 1926. Serial No. 108,417.

This invention relates to improvements in a process for manufacturing solid bodies of cork and the like and has reference to such a process for the production of solid bodies comprising granular particles of cork or other substances which are held together by means of a fresh blood binder or other binding agents.

Heretofore it has not been possible, by 10 the methods employed, to manufacture pressed bodies of granular cork or other substances which possessed a maximum degree of hardness and durability and having a specific gravity equal to that of oak wood 15 or over.

In the processes heretofore employed, and which are outside the scope of this invention, diluted blood albumen or other binding mediums were combined with granulated 20 cork or similar substances and in this wet condition pressed in moulds under pressure of about 16,500 pounds per square inch. Under this high pressure the binder is forced from the core or innermost part of 25 the body toward the surface and even between the walls of the mould and the pressed mass. Due to the applied heat it dries very quickly. The heat acts first to 30 dry the binder near the surface and that portion of the binder which is forced between the mass and the moulds. This produces an air tight jacket or casing around the whole which prevents the drying of the 35 interior of the compressed material, in view of the fact, that the humidity generated by the imprisoned steam is held captive within the mass.

When the said outer jacket is cut or 40 broken away, in products manufactured by the old process just described, it will be found that the inner mass or body crumbles and falls apart due to its still wet condition.

The object of this invention is to overcome 45 the objectional feature above set forth and further to provide a finished product which will possess a maximum hardness and specific gravity equal to that of oak wood, or over.

50 A further object is to provide a process requiring a minimum amount of labor, heat and time to produce the finished product.

The above objects are attained by the method herein described and claimed.

The process embodied in this invention 55 comprises the following various steps:—

The granular cork or substance is thoroughly mixed with a suitable binding medium and is allowed to dry, in its unpressed condition, in the open air. This procedure 60 allows the cells of the granular substance to remain open and permits the entire mass to thoroughly dry throughout. The dried mass of granular particles is then compressed in suitable moulds under pressure 65 of 16,500 pounds per square inch and subjected to a heat up to 130 degrees centigrade.

As soon as the binding medium has reached its melting point, it, especially 70 blood albumen, becomes liquid for the fraction of a second and then hard, so that the actual binding takes only a few minutes according to the size of the mass, whereas heretofore, days were required to dry the 75 product.

While blood albumen is applicable as a binder this invention particularly comprehends the use of fresh blood. Such use is novel in this process and reduces the operations, use of heat, and time necessary to manufacture the finished product, inasmuch as the first stage, namely the mixing of the granular particles and fresh blood, may be accomplished in the vicinity of a slaughterhouse 80 where fresh blood is available. The mixture is then allowed to dry as hereinbefore set forth, after which it may be transported to the point or place where the finished product is made. In this dried 85 form the mass may be stored and permitted to stand for a considerable time as a raw product and without danger of deterioration before shaping or completion.

Another important feature of this invention and novel therein, is the fact that the mixture of granular substance and binder is dried and subsequently this dried mixture is compressed and heated to produce 90 the finished product.

Bodies of granular cork or other substances made in accordance with this invention have been found to possess hardness heretofore never attained and are particularly advantageous for machine pulleys in which use 105 they surpass cast iron pulleys. The product may also be applied as a floor covering or is applicable for numerous other uses.

**What is claimed:**

1. The herein described process for manufacturing articles of pressed granular substances, consisting in mixing a binding medium with granular substances, permitting the substance to dry in the open air and without pressure, compressing the said dried mass under a pressure of 16,500 pounds to the square inch and subjecting same to heat up to 130 degrees centigrade, without re-expansion after release of said pressure and heat.

2. The process set forth in claim 1 wherein the drying and heating is accomplished in a few minutes.

15

3. The process set forth in claim 1, wherein the product is dehydrated to permit storing same as a raw substance for long periods of time.

Signed at New York, in the county of 20  
New York, and State of New York, this  
4th day of May A. D. 1926.

GEORGE SCHELLHAAS.